# EUROPEAN PATENT APPLICATION

(11) **EP 4 327 949 A1**
(43) Date of publication of application: **28.02.2024**
(21) Application number: 23192620.5
(22) Date of filing: 22.08.2023
(51) Int. Cl.: B05B 5/08, B21F 27/00, E04H 17/00, B05D 1/06, B05D 7/14, B05D 7/00, B05D 7/20, B05D 3/04

(54) **METHOD AND APPARATUS FOR COATING A GALVANIZED FENCE PANEL AND THE RESULTING FENCE PANEL**

(30) Priority: 22.08.2022 BE 202205657
(71) Applicant: Balak Coatings nv, 3900 Pelt (BE)
(72) Inventor: van Bakel, Frans, 3900 Pelt (BE); Riepen, Vicky, 3900 Pelt (BE); van Hoeij, Marcel, 3900 Pelt (BE)
(74) Representative: Brantsandpatents bv

(57) **Abstract**

The invention concerns a method for powder coating a galvanized double-wire fencing panel comprising horizontal and vertical wires, wherein the method comprises the steps: feeding the fence panel into two sequential spray booths substantially horizontally, so that a second spray booth is positioned downstream of a first spray booth, wherein a powder is sprayed onto the fence panel in each spray booth by means of spraying means, and wherein the powder adheres to the wires of the fence panel by electrostatic forces; and curing the fence panel in one or more ovens, wherein a coated galvanized fence panel is obtained comprising horizontal wires coated with a first coating thickness and vertical wires coated with a second coating thickness, wherein the ratio of the first and the second coating thickness is between 2.2/1 and 1/2.2. The invention also concerns an apparatus for powder coating a galvanized double-wire fence panel and the resulting coated galvanized double-wire fence panel.

## Description

### TECHNICAL FIELD

The invention relates to a method for coating a galvanized fence panel. The invention also concerns an apparatus for powder coating a galvanized double-wire fence panel and the resulting coated galvanized double-wire fence panel.

### PRIOR ART

Fence panels, and more specifically fence panels for outdoor use, must have sufficient anti-corrosion properties. In addition, fences, for example, must have an aesthetic and beautiful appearance. Applying a powder coating can provide a solution to both problems. By applying a powder coating to a galvanized fence panel, not only a more aesthetic and attractive result is achieved, the corrosion resistance of this so-called duplex system is also considerably better.

A known method for applying a powder coating, as described in JP5721407, consists of preheating the object to be coated to a temperature higher than the melting temperature of the powder. Once the object is hot, it is immediately immersed in a fluidized bed of the powder, whereby the powder melts on contact with the hot object and forms a film. A solid covering is thus obtained. In this process, a hot object is immersed in a cold fluidized bed and to prevent heat loss, an oven with a higher temperature than that required for coating is required, leading to higher energy consumption. Furthermore, if the object consists of parts with very different thermal inertia, these different parts do not have the same temperature and thus the thickness of the film is not uniform. Moreover, the method is not suitable for a continuous powder coating process.

A second known method for electrostatic powdering consists of charging the powder with static electricity and bringing it into contact with the object to be coated, which is connected to a zero potential. For example, the powder is injected into an electrostatic gun that charges the powder by the corona effect (also called crown effect), by triboelectrification or by a combination of the two. The powder thus charged is sprayed onto the object to be covered, which is connected to a zero potential. The guns often need to be set to high spray speeds to achieve the desired coating thickness and uniformity. A problem with the known method is that the high spray speeds are accompanied by high wear of the guns. This results in a frequent need to replace the guns.

The present invention aims to find a solution for at least some of the above problems.

There is a need for an improved method for coating complete galvanized fence panels.

### SUMMARY OF THE INVENTION

The invention concerns a method for coating a galvanized fence panel according to claim 1. Preferred forms of the method are set out in claims 2-14. In a second aspect, the invention concerns a coated galvanized fence panel according to claim 15.

It is an objective of the invention to optimize the coating process for galvanized double-wire fence panels. It is therefore an aim of the invention to obtain a thin coating on the wires of the fence panels over the entire fence panel.

It is also an object of the invention to increase the service life (i.e. the time that it can be in operation) of the spraying means with which the powder is sprayed onto the fence panels. It is therefore also an aim of the invention to reduce the spray speed at which the powder is sprayed onto the fence panel. The aim of a lower spray speed is to significantly reduce wear on the spraying means and significantly increase the lifespan of the spraying means.

Moreover, it is also an aim of the invention to reduce or even avoid losses of raw materials (powder, etc.).

It is a further object of the invention to obtain a uniform coating layer.

### DETAILED DESCRIPTION

The invention concerns a method for coating a galvanized fence panel.

Unless otherwise defined, all terms used in the description of the invention, including technical and scientific terms, have the meaning as commonly understood by a person skilled in the art to which the invention pertains. For a better understanding of the description of the invention, the following terms are explained explicitly.

In this document, "a" and "the" refer to both the singular and the plural, unless the context presupposes otherwise. For example, "a segment" means one or more segments.

When the term "around" or "about" is used in this document with a measurable quantity, a parameter, a duration or moment, and the like, then variations are meant of approx. 20% or less, preferably approx. 10% or less, more preferably approx. 5% or less, even more preferably approx. 1% or less, and even more preferably approx. 0.1% or less than and of the quoted value, insofar as such variations are applicable in the described invention. However, it must be understood that the value of a quantity used where the term "about" or "around" is used, is itself specifically disclosed.

The terms "comprise," "comprising," "provided with," "contain," "containing," "include," "including" are synonyms and are inclusive or open-ended terms that indicate the presence of what follows, and which do not exclude or prevent the presence of other components, characteristics, elements, members, steps, as known from or disclosed in the prior art.

The terms "consist of," "consisting of," "being composed of", "composed of", are synonyms and are exclusive or closed-ended terms indicating the presence of what follows, and excluding or precluding the presence of other components, features, elements, members, steps known or described in the art.

Quoting numeric intervals by the endpoints includes all integers, fractions, and/or real numbers between the endpoints, including those endpoints.

In a first aspect, the invention concerns a method for powder coating a galvanized double-wire fence panel comprising horizontal wires and vertical wires.

In a preferred embodiment the method comprises the steps of:
- feeding the fence panel essentially horizontally into two sequential spray booths, so that a second spray booth is positioned downstream of a first spray booth, wherein powder is sprayed onto the fence panel in each spray booth by means of spraying means, and wherein the powder adheres to the fence panel by electrostatic forces; and
- curing the fence panel in one or more ovens.

In a preferred embodiment the method comprises the steps of:
- feeding the fence panel essentially horizontally into two sequential spray booths, so that a second spray booth is positioned downstream of a first spray booth, wherein powder is sprayed onto the fence panel in each spray booth by means of spraying means, and wherein the powder adheres to the fence panel by electrostatic forces; and
- curing the fence panel in one or more ovens, and
wherein a coated galvanized fence panel is obtained comprising horizontal wires coated with a first coating thickness and vertical wires coated with a second coating thickness, wherein the ratio of the first coating thickness and the second coating thickness is between 2.2/1 and 1/2.2.

It will be apparent to one skilled in the art that the names of the wires in the fence panel, namely "horizontal wires" and "vertical wires," are relative names. The terms "horizontal wires" and "cross wires" refer to the wires or bars which, in a working form (installed condition) of the fence panel, are positioned substantially horizontally with respect to the surface on which the fencing is positioned upright. The horizontal wires therefore correspond to the length of the fence panel. The terms "vertical wires" and "longitudinal wires" refer to the wires or bars that, in a working form (installed condition) of the fence panel, are positioned substantially vertically relative to the surface on which the fencing is positioned upright. The vertical wires therefore correspond to the height of the fence panel. The horizontal wires and vertical wires are thus positioned perpendicular to each other.

When the fence panel is supplied in a substantially horizontal position during coating, both the horizontal wires and the vertical wires lie substantially in a plane parallel to the ground surface, still positioned perpendicular to each other.

In a preferred form, the fence panel is coated in a substantially horizontal position. In a further preferred form, the fence panel is positioned for this purpose on at least 4 support points. At least four support points are needed for the horizontal positioning of the fence panel without it becoming crooked or unstable. Furthermore, the number of support points is preferably minimized. This minimizes the number of contact points and possible irregularities in the coating.

The fence panel is preferably positioned on a maximum of 12 support points, preferably a maximum of 9, even more preferably a maximum of 8, even more preferably a maximum of 5.

"The support points" are defined as positions on the fence panel that contact a support means. The fence panel is preferably provided with zero potential via these support points, i.e. the fence panel is earthed via these support points. A set of support points is a set of positions on the fence panel that contact a support means.

In an embodiment, the fence panel in the first and the second spray booth are positioned on the same set of support points.

In an alternative embodiment, the fence panels are positioned in the first spray booth on a first set of support points, and in the second spray booth positioned on a second set of support points, wherein the first set of support points and the second set of support points are different, i.e. do not have any support points in common.

This is possible by, in an embodiment, moving or shifting the fence panel horizontally relative to the support means, so that a new set of support points is formed. Alternatively, this is possible by turning the fence panel over, so that a new set of support points is formed on the opposite side face of the twin-wire fence panel.

This prevents no coating from ending up on the contact points made by the fence panel on the support points during spraying, requiring manual touch-ups afterwards.

The method optimizes the coating process for galvanized double-wire fence panels. So that a thin coating can be obtained over the entire fence panel. The method is advantageous because a lower spray speed can be used, which significantly reduces wear on the spraying means and significantly increases the lifespan of the spraying means.

Preferably the method takes place continuously.

In a specific preferred form, a maximum of one fence panel is coated at a time (per spray booth). The fence panels pass through the booths individually and not in a plurality, which is the usual method in the prior art. This method is advantageous because the coating layer thickness per fence panel and at different locations on each fence panel can be controlled/realized much more accurately. In a process in which the fence panels are coated "in a package" or in a plurality, much more powder must be sprayed to achieve sufficient coating thickness also on the inside of the package.

In an embodiment, the fence panel is made of unalloyed steel, low-alloy steel or high-alloy steel. The fence panel can be manufactured from high or low carbon steel.

Unalloyed steel contains a maximum of 1.5% of alloying elements (excluding carbon (C)). Unalloyed steel has a carbon percentage of 0.5% to 2%. Low-alloy steel contains between 1.5 and 5% alloying elements (excluding carbon). High-alloy steel contains more than 5% of alloying elements. The fence panel is preferably made of unalloyed steel. The term "alloying elements" refers to the elements that are present in the alloy in addition to iron and carbon. In a preferred form, the fence panel is made of an alloy comprising iron (Fe), carbon (C) and alloying elements. Preferably, the alloy comprises a maximum of 1.5% alloying elements, more preferably a maximum of 1.4%, even more preferably a maximum of 1.3%, even more preferably a maximum of 1.2%, most preferably a maximum of 1.1%. Preferably the alloy comprises at least 0.5% alloying elements, more preferably at least 0.6%, even more preferably at least 0.7%, even more preferably at least 0.8%, even more preferably at least 0.9%, most preferably at least 1%. In another preferred embodiment, the alloy comprises between 0.5 and 1.5% alloying elements, preferably between 0.6 and 1.5%, more preferably between 0.7 and 1.4%, even more preferably between 0.8 and 1.3%, even more preferably between 0.9 and 1.2%, most preferably between 1 and 1.1%.

In an embodiment, the alloy comprises a maximum of 0.1% C, more preferably a maximum of 0.09%, even more preferably a maximum of 0.085%, even more preferably a maximum of 0.08%, most preferably a maximum of 0.075%. Preferably, the alloy comprises at least 0.025% C, more preferably at least 0.03%, even more preferably at least 0.035%, even more preferably at least 0.04%, most preferably at least 0.045%. In another preferred embodiment, the alloy comprises between 0.02 and 0.1% C, preferably between 0.025 and 0.09%, more preferably between 0.035 and 0.085%, even more preferably between 0.04 and 0.08%, most preferably between 0.045 and 0.075%.

In a preferred embodiment, the alloy comprises alloying elements selected from the list of: manganese (Mn), silicon (Si), sulfur (S), phosphorus (P), nitrogen (N), copper (Cu), chromium (Cr), nickel (Ni), niobium (Nb), tin (Sn), aluminum (Al) or any combination thereof. Preferably the alloy comprises manganese (Mn), silicon (Si), sulfur (S), phosphorus (P), nitrogen (N), copper (Cu), and optionally chromium (Cr), nickel (Ni), niobium (Nb), tin (Sn), aluminum (Al).

Preferably, the alloy comprises Mn in an amount between 0.3 and 0.5%, more preferably between 0.35 and 0.45%, Si in an amount between 0.05 and 0.25%, more preferably between 0.1 and 0.2%, S in an amount between 0.01 and 0.045%, more preferably between 0.015 and 0.04%, P in an amount between 0.005 and 0.03%, more preferably between 0.005 and 0.025%, Cu in an amount between 0.2 and 0.4%, more preferably between 0.25 and 0.35%, N in an amount between 0.005 and 0.02%, more preferably between 0.005 and 0.015%, and Cr in an amount of up to 0.15%, more preferably up to 0.1%, Ni in an amount up to 0.15%, more preferably up to 0.1%, and Nb in an amount up to 0.005%, more preferably up to 0.002%, Sn in an amount up to 0.05%, more preferably up to 0.03%, and/or Al in an amount up to 0.005%, more preferably up to 0.003%.

In a preferred form, the fence panel is a twin-wire or double-wire fence panel. With double-wire fence panels, parallel vertical bars (wires) are welded to horizontal bars (wires), whereby the vertical bars are welded at the same height between two horizontal bars (a pair). The fence panel preferably has between 50 and 55, preferably 51, vertical bars and between 1 and 20 horizontal bars.

In an embodiment, the vertical wires have a length between 500 and 2500 mm, preferably the vertical wires have a length selected from the list: 630, 830, 1030, 1230, 1430, 1630, 1830, 2030, 2230, 2430 mm. It will be apparent to one skilled in the art that the length of the vertical wires corresponds to the height of a fence panel. In an embodiment, the horizontal wires have a length between 2000 and 3000 mm; preferably between 2400 and 2600, even more preferably between 2500 and 2550 mm, most preferably 2508 or 2510 mm. It will be apparent to one skilled in the art that the length of the horizontal wires corresponds to the length of a fence panel.

In a preferred embodiment, the distance between two adjacent vertical wires is 40-60 mm c.t.c., more preferably between 45 and 55 mm, even more preferably between 49 and 51, most preferably about 50 mm.

In another embodiment, the distance between the adjacent horizontal wires is 100-300 mm c.t.c., preferably 150-250 mm, more preferably 180-220 mm, most preferably about 200 mm.

The term "c.t.c." (center to center) refers to a distance between the center (the heart) of a circular cross-section of one wire and the center (the heart) of a circular cross-section of another wire.

In an embodiment, the fence panel is galvanized prior to coating. In a preferred form, the fence panel is hot-dip galvanized, whereby a zinc layer is deposited on the fence panel. In a further preferred form, the fence panel is provided with a zinc layer with a thickness between 40 and 120 mu. In a further or other preferred form, the average thickness of the zinc layer on the wires of the fence panel is between 60 and 80 mu.

Applying a powder coating to a galvanized fence panel not only produces a more aesthetically pleasing result, but also significantly improves the corrosion resistance of the fence panel. Zinc is one of the most difficult surfaces to apply a paint system to. The reason for this is that the quality of the hot-dip galvanized material can vary greatly. In addition, many contaminants can occur on the zinc surface, such as corrosion products, passivation layers on sendzimir galvanized steel, rolling oil, etc. In a further or different embodiment, the fence panel is therefore pre-treated prior to coating. The pre-treatment preferably comprises one or more steps from the list of: degreasing, rinsing, demi-rinsing, pickling, fluxing, demi-fogging, conversion coating, such as phosphating, zirconizing, chromating, passivating, iron phosphating, zinc phosphating, manganese phosphating, stove-enameling, or a combination of these. In a preferred form, the fence panel is pretreated through the steps of: degreasing, rinsing, demi-rinsing, pickling, fluxing, applying a conversion layer, curing, or a combination of these.

Preferably, the fence panel is provided in the pre-treatment with a conversion layer or adhesion layer that is formed on the metal surface by the action of a chemical agent, such as a polymer.

In an embodiment, the fence panel is supplied essentially horizontally into two sequential spray booths, so that a second spray booth is positioned downstream of a first spray booth.

Feeding preferably takes place by means of guide means which guide the fence panel substantially horizontally through the first and then through the second spray booth. The guide means preferably make a minimum number of contact points with the fence panel or have a minimum contact surface with the fence panel. This is because the contact points ensure that the fence panel cannot be covered with powder in those areas. Therefore, the guide means can for instance comprise two narrow guide means, such as conveyor belts, which support two opposite sides of a fence panel.

In an embodiment, the guide means are suitable for advancing the fence panels through the spray booths at a constant speed between 1 and 10 m/min, preferably between 5 and 7.5 m/min.

The fence panel is grounded, i.e. connected to zero potential, before spraying the powder.

In an embodiment, powder and therefore powder particles are sprayed onto the fence panel in each spray booth using spraying means. The powder adheres to the fence panel by electrostatic forces. The powder particles are transported by an air stream to the spraying means. They acquire an electrostatic charge and thus adhere to the grounded fence panel through electrostatic forces. In a preferred form, the spraying means sprays the powder in an upward vertical direction perpendicular to the horizontal plane, i.e. the opposite direction of gravity. In this process, the powder is atomized into a powder cloud through which the fence panels move.

In an embodiment, the charge is applied to the powder by an electrode where a discharge takes place (= corona principle), or by friction along a non-conductive material (tribo principle), preferably the charge is applied using the tribo principle by a tribo-charging system. The tribo principle is advantageous because the effect of a Faraday cage can be avoided.

The spraying means are preferably spray guns, more preferably the spraying means are triboelectric powder coating guns. The tribo-gun contains a friction system through which powder is guided and that comes out of the gun positively charged.

In a preferred embodiment, the spraying means spray the powder onto the fence panel at a spraying speed of 2-8 m/min, preferably 3-7 m/min, more preferably 4-6 m/min.

The spray speed of the spraying means can also be expressed on the basis of powder consumption. In a preferred form the spraying means sprays the powder onto the fence panel at a spray speed between 1 and 100 g/min, preferably between 10 and 50 g/min, more preferably between 20 and 45 g/min, even more preferably between 30 and 40 g/min, and most preferably between 35 and 40 g/min. Here, g/min refers to the number of grams of powder that is sprayed onto the fence panel per minute per spraying means.

In another embodiment, the fence panels are provided with powder at a rate of between 3 and 10 m²/min, preferably between 4 and 9 m²/min, more preferably between 5 and 8 m²/min, even more preferably between 6 and 7 m²/min. Where m²/min refers to the full surface of the fence panel that is provided with powder per minute.

The use of two booths ensures that the layer thickness can be better controlled. As a result, the spraying means also have to process less powder per time unit, so that the spraying means last longer.

The powder comprises one or more components that form a protective coating on the object when heated. Powders can be, for example, polyamides, polyolefins, epoxies, polyesters, or a combination of these.

Polyamides are condensation products of one or more amino acids, such as aminocaproic acid, amino-7-heptanoic acid, amino-11-undecanoic acid and amino-12-dodecanoic acid, or of one or more lactams, such as caprolactam, oenantholactam and lauryllactam, or of one or more salts or mixtures of diamines such as hexamethylenediamine, dodecamethylenediamine, metaxylenediamine, bis-p aminocyclohexylmethane and trimethylhexamethylenediamine with diacids such as isophthalic acid, terephthalic acid, adipic acid, azelaic acid, suberic acid, sebacic acid and dodecanedioic acid or mixtures of all these monomers, which lead to copolyamides.

Polyolefins are understood to mean polymers containing olefin units, such as, for example, ethylene, propylene, butene-1 units. Examples of polyolefins are:
- polyethylene, polypropylene, copolymers of ethylene with alpha-olefins. These products can be grafted with anhydrides of unsaturated carboxylic acids such as maleic anhydride or unsaturated epoxides such as glycidyl methacrylate, and
- copolymers of ethylene with at least one product selected from i) unsaturated carboxylic acids, their salts and esters, ii) vinyl esters of saturated carboxylic acids, iii) unsaturated dicarboxylic acids, their salts, esters, hemiesters and anhydrides, and iv) the unsaturated epoxides. These ethylene copolymers can be grafted with anhydrides of unsaturated dicarboxylic acids or unsaturated epoxides.

Polyesters can be chosen from the list of: poly(3-hydroxybutyrate-co-3-hydroxyvalerate), poly(lactic acid-co-glycolic acid), poly(ethylene succinate), polybutylene adipate terephthalate, polybutylene succinate, polybutylene terephthalate, polycaprolactone, polycyclohexylenedimethylene terephthalate, polydioxanone, polyethylene naphthalate, polyethylene terephthalate, polyglycolide, polyhydroxyalkanoates, polyhydroxybutyrate, polylactic acid, polytrimethylene terephthalate.

In a preferred form the powder comprises polyester, preferably the powder comprises a polyester selected from the list of: polybutylene succinate, polybutylene terephthalic acid, polycaprolactone, polyethylene naphthalate, polyethylene terephthalate, polyglycolide, polyhydroxyalkanoates, polyhydroxybutyrate, polylactic acid. This is advantageously a polyester resin.

In an embodiment, the D50 particle size of the powder is between 1 and 100 µm, preferably between 10 and 90 µm, more preferably between 20 and 80 µm, even more preferably between 30 and 70 µm, even more preferably between 40 and 60 µm, most preferably between 45 and 55 µm.

In an embodiment, a coated galvanized fence panel is obtained with a coating thickness between 25 and 150 mu. In a further embodiment, a coated galvanized fence panel is obtained, wherein the vertical wires have a coating thickness between 50 and 150 mu, preferably between 60 and 140 mu, more preferably between 70 and 130 mu, even more preferably between 80 and 120 mu, even more preferably between 90 and 110 mu, most preferably between 95 and 105 mu, most preferably about 100 mu. In a further embodiment, the horizontal wires have a coating thickness between 25 and 75 mu, preferably between 30 and 70 mu, more preferably between 35 and 65 mu, even more preferably between 40 and 60 mu, even more preferably between 45 and 55 mu, most preferably between 50 mu.

In a preferred form, prior to feeding the fence panel into the second spray booth, the powder adhered to the vertical wires is blown away using air lances. In this case, the air lances are preferably only aimed at the vertical wires. In an embodiment, the powder is blown off all vertical wires simultaneously. In another embodiment, the powder is blown off the vertical wires one by one.

The preferred form is advantageous because the powder attached to the vertical wires is blown away by means of air lances after the first spray booth, so that a more uniform and thinner layer is obtained after spraying in the second spray booth. A substantially equal coating thickness is hereby obtained on the vertical and horizontal wires.

In a preferred embodiment, approximately all of the powder on the vertical wires is blown away, so that the thickness of the coating present on the vertical wires after blowing is a maximum of 5 mu, preferably a maximum of 4 mu, more preferably a maximum of 3 mu, even more preferably maximum 2 mu, most preferably maximum 1 mu.

In a further preferred embodiment, the air blown out of the air lances has a pressure between 1 and 2 bar, preferably between 1 and 1.25 bar, more preferably about 1 bar.

In another or further preferred embodiment, the air is blown out of the air lances at a flow rate of between 100 and 400 m³/hour, preferably between 150 and 350 m³/hour, more preferably between 200 and 300 m³/hour.

In an embodiment, a coated galvanized fence panel can thus be obtained with a coating thickness between 25 and 150 mu. In a further embodiment, a coated galvanized fence panel is obtained, wherein the vertical wires have a coating thickness between 25 and 75 mu, preferably between 30 and 70 mu, more preferably between 35 and 65 mu, even more preferably between 40 and 60 mu, even more preferably between 45 and 55 mu, most preferably between 50 mu. In a further embodiment, the horizontal wires have a coating thickness between 25 and 75 mu, preferably between 30 and 70 mu, more preferably between 35 and 65 mu, even more preferably between 40 and 60 mu, even more preferably between 45 and 55 mu, most preferably between 50 mu.

In a preferred embodiment, the ratio of the coating thickness on the vertical wires to the coating thickness on the horizontal wires is at most 2.2/1, preferably at most 2/1, more preferably at most 1.8/1, even more preferably at most 1.6/1, even more preferably at most 1.4/1, even more preferably at most 1.2/1, most preferably at most 1.1/1. In a further or other preferred embodiment, the ratio of the coating thickness on the vertical wires to the coating thickness on the horizontal wires is at least 1/2.2, preferably at least 1/2, more preferably at least 1/1.8, even more preferably at least 1/1.6, even more preferably at least 1/1.4, even more preferably at least 1/1.2, most preferably at least 1/1.1. In a further preferred embodiment, the ratio of the coating thickness on the vertical wires to the coating thickness on the horizontal wires is between 2.2/1 and 1/2.2, preferably between 2/1 and 1/2, more preferably between 1.8/1 and 1/1.8, even more preferably between 1.6/1 and 1/1.6, even more preferably between 1.4/1 and 1/1.4, even more preferably between 1.2/1 and 1/1.2, most preferably between 1.1/1 and 1/1.1.

In a further preferred form, the average thickness of the coating on the entire fence panel is 30-70 mu, preferably 40-60 mu, more preferably between 45 and 55 mu, most preferably about 50 mu.

In an embodiment, the method comprises curing the fence panel in one or more ovens. The powder melts in the oven so that it can then harden and form a coating.

In an embodiment, curing is applied to a plurality of fence panels. In a preferred form, between 2 and 100 fence panels are cured at the same time, preferably between 10 and 90, more preferably between 20 and 80, even more preferably between 30 and 70, most preferably between 40 and 60. In case the process takes place continuously, it will be apparent to one skilled in the art that in each oven between 1 and 100 fence panels, preferably between 5 and 80, more preferably between 10 and 60, even more preferably between 15 and 40, most preferably between 20 and 30, are powdered at the same time. In this embodiment, the fence panels are stacked horizontally on top of or below each other with a space in between after the second spray booth.

In a preferred form, a plurality of parallel stacked horizontally positioned fence panels are cured simultaneously.

In a preferred form, the curing of the fence panels takes place in one or two ovens, preferably two ovens, most preferably two sequential ovens, whereby the fence panels are cured in a first oven and then cured in a second oven.

In a preferred form, the fence panel is cured in two sequential (series-connected) ovens. In a further preferred form, the fence panel is introduced into a first oven by means of a vertical upward or downward movement and introduced into a second oven by means of a horizontal movement.

In a preferred form, the fence panel has a residence time between 5 and 15 minutes, preferably between 8 and 12 minutes per oven.

In a preferred form, the one or more ovens operate at an air temperature between 200 and 260°C, preferably between 210 and 250°C, more preferably between 220 and 240°C.

In an embodiment, the fence panels are visually inspected after curing by one or more operators and/or checked using a layer thickness gauge.

In an embodiment, the places on the fence panel where insufficient coating has been applied, such as the contact points that the fence panel made with the guide means, are manually corrected with paint coating.

In an embodiment, a third spray booth is added to the method downstream of the second spray booth, whereby the fence panel is provided with powder a third time, so that the spray speed of the spraying means can be further reduced.

In a second aspect, the invention concerns an apparatus for powder coating a galvanized double-wire fence panel comprising horizontal wires and vertical wires.

In a preferred embodiment the apparatus comprises:
- a first spray booth comprising:
   ∘ a first spraying system comprising spraying means suitable for electrostatically charging a powder,
- a second spray booth comprising:
   ∘ a second spraying system comprising spraying means suitable for electrostatically charging a powder,
wherein the first and the second spray booth are connected in series, so that the second spray booth is positioned downstream of the first spray booth, wherein the first and the second spray booth are provided with at least 4 support means suitable for horizontally supporting the fence panel.

At least four support points are needed for the horizontal positioning of the fence panel without it becoming crooked or unstable. Furthermore, the number of support means is preferably minimized. This minimizes the number of support points and possible irregularities in the coating.

The first and the second spray booth are preferably provided with a maximum of 12 support means, preferably a maximum of 9, even more preferably a maximum of 8, even more preferably a maximum of 5.

In a further preferred form, the apparatus comprises a guide system for guiding a substantially horizontal fence panel through the first and second spray booth. The guide system is preferably provided with at least 4 support means suitable for horizontally supporting the fence panel.

The guide system is preferably provided with a maximum of 12 support means, preferably a maximum of 9, even more preferably a maximum of 8, even more preferably a maximum of 5.

In a preferred embodiment the apparatus comprises:
- a first spray booth comprising:
   ∘ a first spraying system comprising spraying means suitable for electrostatically charging a powder,
   ∘ a first guide system comprising for guiding a substantially horizontal fence panel through the spray booth,
- a second spray booth comprising:
   ∘ a second spraying system comprising spraying means suitable for electrostatically charging a powder,
   ∘ a second guide system comprising guide means for guiding a substantially horizontal fence panel through the spray booth, and
- one or more muffle furnaces,
wherein the first and the second spray booths are connected in series, so that the second spray booth is positioned downstream of the first spray booth, wherein the first and second guidance systems have substantially the same conduction speed.

In a preferred form, the apparatus further comprises a blowing apparatus comprising air lances and a third guide system, wherein the blowing apparatus is positioned between the first and second spray booth and wherein the first, the second and the third guide systems have substantially the same guiding speed.

In a preferred form, the first and second guide systems comprise at least four support means suitable for horizontally supporting the fence panel. At least four support means are required to position the fence panel horizontally without it becoming crooked or unstable. Furthermore, the number of support means is preferably minimized. This minimizes the number of support points and possible irregularities in the coating.

Preferably, the first and second guide systems comprise a maximum of 12 support means, preferably a maximum of 9, even more preferably a maximum of 8, even more preferably a maximum of 5.

In an embodiment, the support means of the first and second guide systems are positioned differently from each other. So that on the first and second guide systems the support means make contact with different parts of the fence panel. This means that the orientation of the support means relative to each other in the first and second guide systems are different.

In a preferred form, the apparatus is suitable for carrying out a method according to the first aspect.

In a third aspect, the invention concerns a coated galvanized double-wire comprising horizontal wires and vertical wires.

In a preferred embodiment, the thickness of the coating on the vertical and horizontal wires is between 25 and 150 mu.

In a further embodiment, the vertical wires have a coating thickness between 25 and 75 mu, preferably between 30 and 70 mu, more preferably between 35 and 65 mu, even more preferably between 40 and 60 mu, even more preferably between 45 and 55 mu, most preferably between 50 mu. In a further embodiment, the horizontal wires have a coating thickness between 25 and 75 mu, preferably between 30 and 70 mu, more preferably between 35 and 65 mu, even more preferably between 40 and 60 mu, even more preferably between 45 and 55 mu, most preferably between 50 mu.

In a preferred embodiment, the ratio of the coating thickness on the horizontal wires to the coating thickness on the vertical wires is at most 2.2/1, preferably at most 2/1, more preferably at most 1.8/1, even more preferably at most 1.6/1, even more preferably at most 1.4/1, even more preferably at most 1.2/1, most preferably at most 1.1/1. In a further or other preferred embodiment, the ratio of the coating thickness on the horizontal wires to the coating thickness on the vertical wires is at least 1/2.2, preferably at least 1/2, more preferably at least 1/1.8, even more preferably at least 1/1.6, even more preferably at least 1/1.4, even more preferably at least 1/1.2, most preferably at least 1/1.1. In a further preferred form, the ratio of the coating thickness on the horizontal wires to the coating thickness on the vertical wires is between 2.2/1 and 1/2.2, preferably between 2/1 and 1/2, more preferably between 1.8/1 and 1/1.8, even more preferably between 1.6/1 and 1/1.6, even more preferably between 1.4/1 and 1/1.4, even more preferably between 1.2/1 and 1/1.2, most preferably between 1.1/1 and 1/1.1.

In a preferred form, the fence panel is obtained according to a method of the first aspect.

In what follows, the invention is described by way of non-limiting examples illustrating the invention, and which are not intended to and should not be interpreted as limiting the scope of the invention.

### EXAMPLES AND DESCRIPTION OF THE FIGURES

**Figure 1** shows a perspective view of a double-wire fence panel.
**Figure 2** shows an enlarged perspective view of a double-wire fence panel (section A in **Figure 2****).**

**Example 1** concerns a twin-wire fence panel, as shown in **Figure 1** and **Figure 2****,** which can be coated according to the method of the first aspect.

A twin-wire fence panel (108) consists of parallel vertical wires (104) welded to horizontal wires (101, 102) with the vertical wires welded at any height between two horizontal wires (101, 102) forming a double pair (103). The distance between two adjacent vertical wires (106) is about 50 mm c.t.c. The distance between the adjacent horizontal wires (105) is about 200 mm c.t.c.

It will be apparent to one skilled in the art that the names of the wires in the fence panel, namely "horizontal wires" and "vertical wires," are relative names. The terms "horizontal wires" and "cross wires" refer to the wires or bars which, in a working form (installed condition) of the fence panel, are positioned substantially horizontally with respect to the surface on which the fencing is positioned upright. The horizontal wires therefore correspond to the length of the fence panel. The terms "vertical wires" and "longitudinal wires" refer to the wires or bars that, in a working form (installed condition) of the fence panel, are positioned substantially vertically relative to the surface on which the fencing is positioned upright. The vertical wires therefore correspond to the height of the fence panel. The horizontal wires and vertical wires are thus positioned perpendicular to each other.

When the fence panel is positioned substantially horizontally during coating, both the horizontal wires and the vertical wires lie substantially in a plane parallel to the ground surface, still positioned perpendicular to each other.

**Example 2** concerns an embodiment of the method according to the first aspect. A pre-treated and galvanized double-wire fence panel is supplied essentially horizontally to a first spray booth in which polyester in powder form, with D50 = 50 µm, is sprayed onto the fence panel using triboelectric powder coating guns, so that the powder is electrically charged through the triboelectric effect. The fence panel is grounded, i.e. connected to zero potential, before spraying the powder. The guns spray the powder onto the fence panel at a spray speed of 4-6 m/min. The fence panel remains in the first spray booth for between 20 and 28 seconds. The fence panel is then transported to a second spray booth. The guns spray the powder onto the fence panel at a spray speed of 4-6 m/min. The fence panel remains in the first spray booth for between 20 and 28 seconds. A coated galvanized fence panel is obtained comprising horizontal wires coated with a thickness of approximately 50 mu and vertical wires coated with a thickness of approximately 100 mu.

**Example 3** concerns an embodiment of the method according to the first aspect. A pre-treated and galvanized double-wire fence panel is supplied essentially horizontally to a first spray booth in which polyester in powder form, with a D50 = 50 µm, is sprayed onto the fence panel using triboelectric powder coating guns, so that the powder is electrically charged through the triboelectric effect. The fence panel is grounded, i.e. connected to zero potential, before spraying the powder. The guns spray the powder onto the fence panel at a spray speed of 4-6 m/min. The fence panel remains in the first spray booth for between 20 and 28 seconds. The powder then adhered to the vertical wires is then blown away so that a maximum of 1 mu of powder is present on the vertical wires. The fence panel is then transported to a second spray booth. The triboelectric powder coating guns spray the powder onto the fence panel at a spray speed of 4-6 m/min. The fence panel remains in the first spray booth for between 20 and 28 seconds. A coated galvanized fence panel is obtained comprising horizontal wires coated with a thickness of approximately 50 mu and vertical wires coated with a thickness of approximately 50 mu.

The present invention should not be construed as being limited to the embodiments described above and certain modifications or changes may be added to the examples described without having to re-evaluate the appended claims. For example, the present invention has been described with reference to a double-wire fence panel with seven pairs of horizontal wires, but it should be understood that the invention can be applied to, for example, a fence panel with 7 pairs of horizontal wires or 1, 2, 3, 4, 5, 6, 8, 9, 10, 11, 12, 13, 14, 15, 16, 17, 18, 19, 20 pairs of horizontal wires.

## Claims

1. A method of powder coating a galvanized double-wire fence panel comprising horizontal wires and vertical wires, the method comprising the steps of:
- feeding the fence panel essentially horizontally into two sequential spray booths, so that a second spray booth is positioned downstream of a first spray booth, wherein a powder is sprayed onto the fence panel in each spray booth by means of spraying means, and wherein the powder adheres to the wires of the fence panel by electrostatic forces; and
- curing the fence panel in one or more ovens;
wherein the spraying means are triboelectric powder coating guns, so that the powder is electrically charged through the triboelectric effect.

2. Method according to claim 1, wherein a maximum of one fence panel is coated per spray booth.

3. Method according to claim 1 or 2, wherein the spraying means spray the powder onto the fence panel at a spray speed between 1 and 100 g/min.

4. Method according to any one of the preceding claims, wherein the spraying means spray the powder onto the fence panel at a spray speed between 30 and 40 g/min.

5. Method according to any one of the preceding claims, wherein the fence panel remains in a spray booth between 15 and 35 s, preferably between 20 and 30 s.

6. Method according to any one of claims 4-6, wherein the thickness of the coating on the wires of the fence panel is 30-70 mu, preferably 40-60 mu.

7. Method according to any one of the preceding claims, wherein the coating is a polyester coating.

8. Method according to any one of the preceding claims, wherein the curing of the fence panel takes place in two ovens, preferably two sequential ovens.

9. Method according to any one of the preceding claims, wherein a plurality of parallel stacked, horizontally positioned fence panels are simultaneously cured.

10. Method according to any one of the preceding claims, wherein the fence panel is positioned on at least 4 support points during coating.

11. Method according to any one of the preceding claims, wherein the fence panel is positioned on between 4 and 9 support points during coating.

12. An apparatus for powder coating a galvanized double-wire fence panel comprising horizontal wires and vertical wires, the apparatus comprising:
- a first spray booth comprising:
∘ a first spraying system comprising spraying means suitable for electrostatically charging a powder,
- a second spray booth comprising:
∘ a second spraying system comprising spraying means suitable for electrostatically charging a powder,
wherein the first and the second spray booth are connected in series, so that the second spray booth is positioned downstream of the first spray booth, wherein the first and the second spray booth are provided with at least 4 support means suitable for horizontally supporting the fence panel.

13. Apparatus according to claim 12, wherein the apparatus comprises:
- a first spray booth comprising:
∘ a first spraying system comprising spraying means suitable for electrostatically charging a powder,
∘ a first guide system comprising for guiding a substantially horizontal fence panel through the spray booth,
- a second spray booth comprising:
∘ a second spraying system comprising spraying means suitable for electrostatically charging a powder,
∘ a second guide system comprising guide means for guiding a substantially horizontal fence panel through the spray booth,
wherein the first and the second spray booths are connected in series, so that the second spray booth is positioned downstream of the first spray booth, wherein the first and second guide systems have substantially the same conduction speed.

14. Apparatus according to claim 13, wherein the first and second guide system each comprise at least 4 support means suitable for horizontally supporting the fence panel.

15. A coated galvanized double-wire fence panel comprising horizontal wires provided with a coating with a first coating thickness and vertical wires provided with a coating with a second coating thickness, **characterized in that** the ratio of the first coating thickness to the second coating thickness is between 2.2 /1 and 1/1.
